

[54] METHOD FOR FABRICATING A BERYLLIUM FIBER REINFORCED COMPOSITE HAVING A TITANIUM MATRIX

[75] Inventor: Vernon L. Goodwin, Willowick, Ohio

[73] Assignee: Brush Wellman Inc., Cleveland, Ohio

[22] Filed: Aug. 18, 1972

[21] Appl. No.: 281,620

[52] U.S. Cl..... 29/419, 29/182.2, 29/420.5, 29/DIG. 45, 29/DIG. 47, 75/226

[51] Int. Cl..... B22f 3/24, B23p 17/00

[58] Field of Search. 29/DIG. 31, DIG. 45, DIG. 47, 29/419, 420, 420.5, 182.2; 75/200, 226

[56] References Cited

UNITED STATES PATENTS

|           |         |                     |            |
|-----------|---------|---------------------|------------|
| 2,940,163 | 6/1960  | Davies .....        | 29/182.2   |
| 3,390,985 | 7/1968  | Croeni et al.....   | 29/420.5 X |
| 3,475,142 | 10/1969 | Abkowitz et al..... | 29/420.5 X |
| 3,510,275 | 5/1970  | Schwope et al.....  | 29/419 X   |
| 3,609,855 | 10/1971 | Schmidt.....        | 29/420.5 X |
| 3,667,108 | 6/1972  | Schmidt.....        | 29/DIG. 45 |
| 3,681,037 | 8/1972  | Abkowitz et al..... | 75/226 X   |

Primary Examiner—Charles W. Lanham

Assistant Examiner—D. C. Reiley, III

Attorney, Agent, or Firm—McNenny, Farrington, Pearne & Gordon

[57]

ABSTRACT

A process for forming fibrous beryllium/titanium composites from separate beryllium and titanium materials wherein the resultant composite consists of continuous Be fibers of selective size, array, placement, and geometry in a matrix of continuous Ti or Ti alloy phase. The process is characterized by surrounding discrete preformed Be shapes or fiber precursor bodies with either powdered or preformed Ti material and extruding a cannister containing this assembled body at a temperature of from 1,350° to 1,525°F. to a reduction ratio of from 6/1 to 100/1 or greater to form a consolidated Be/Ti composite having a very limited but discernible intermetallic reaction zone of titanium beryllide formed in situ. After extrusion and cooling, the yield strength of the composite can, if desired, be substantially improved by cold working at 70% to 80% of the ultimate tensile strength. Composite beryllium titanium bodies so fabricated have tensile properties superior to those of Be/Ti composites fabricated up to 1,300°F. and superior ductility, toughness and strength to those of Be/Ti composites made from blended Be and Ti powders hot extruded at 1,350°F. to 1,525°F. Furthermore, because of the capability of controlling the geometry of the array of fibers in composite sections, it is possible to "design" properties to specific applications. These materials may be fabricated by known techniques into aircraft engine parts, e.g., gas turbine compressor blades, vanes and shafts. They would also be useful in other shaft applications requiring high modulus and low weight such as high speed machinery.

20 Claims, 5 Drawing Figures



PATENTED JUL 2 1974

3,821,841

SHEET 1 OF 2

*Fig. 1*



*Fig. 2*

PATENTED JUL 2 1974

3,821,841

SHEET 2 OF 2

*Fig. 3*



*Fig. 4*



*Fig. 5*



**METHOD FOR FABRICATING A BERYLLIUM  
FIBER REINFORCED COMPOSITE HAVING A  
TITANIUM MATRIX**

**BACKGROUND OF THE INVENTION AND PRIOR  
ART**

Beryllium metal has the advantage of possessing one of the higher specific elastic moduli (elastic modulus/density) of any existing metal. However, opposing disadvantages are the low fracture toughness and high fabricating costs. Thus, the use of beryllium as a structural metal has been limited. Titanium and its alloys in contrast have good specific strength (strength/density) and acceptable fracture toughness properties, but a lower than desired elastic modulus. Alloys containing substantial amounts of Be and Ti prepared by conventional melting practices cannot avoid the formation of excessive amounts of brittle intermetallic reaction products which cause the overall alloy to be uselessly brittle.

By this invention, Be and titanium materials can be bonded together and mutually reinforced by permitting a limited interaction between contacting areas of adjacent Be-Ti material to form an amount of titanium beryllide sufficient to join strongly together, but insufficient to interfere with the desirable individually contributed properties of the Be and Ti and render the product brittle. Fabrication of Be/Ti composites has already been investigated and reported by Abkowitz in U.S. Pat. No. 3,475,142. Schmidt in U.S. Pat. No. 3,609,855 describes a method of hot rolling assemblies of Be/Ti into composite ribbon. Abkowitz limited the temperature of processing treatment to 1,300°F. and below in order to ensure against the formation of titanium beryllide interaction products between beryllium and titanium particles. Such intermetallic structures are recognized as being brittle and causing nonductile bonds leading to premature failure under stressing. The present work has found in processing from 1,375°F. and higher that fibrous composite bodies were formed exhibiting greater tensile ductility than those fabricated at 1,300°F. and below. Also, higher strength resulted in processing composite beryllium/titanium material in the range of 1,375° to 1,525°F. This is contrary to the art taught by Abkowitz and to that generally recognized presently by material scientists. Metallographic examination at 500 - 10,000X of beryllium/titanium composites made by processing powder blends from 1,100° - 1,525°F. showed no evidence of significant interparticle titanium beryllide reaction at 1,300°F. and below, but did find evidence of some at 1,375°F. and above, the reaction zone being thicker with higher temperatures and longer times of exposure at these temperatures.

The present work departs from that of Schmidt in that he uses exclusively the process of hot rolling and is concerned with fabricating composite ribbon only.

One purpose of the present invention is to provide a beryllium/titanium composite material having a modulus of elasticity substantially greater than that of titanium ( $16 \times 10^6$  psi), a density similar to or slightly greater than that of aluminum (0.100 to 0.135 lb. per cubic inch), a tensile ductility in the longitudinal direction of 2% or greater combined with a transverse direction elongation of 1.0% or greater, and a notched Charpy impact strength of 5 foot pounds or greater at room temperature. These characteristics are considered by aircraft manufacturers to be worthy properties

for aircraft structural elements. Also, a family of applications exist wherein Be/Ti fibrous composites can be produced as shafting and used to replace steel and other commonly used shaft materials which are relatively heavy compared to Be/Ti composites. The advantage of a low density material with a modulus of elasticity comparable to steel is that the resonant frequency of the shaft is increased, thereby allowing the shaft to operate at higher speeds than steel shafts before excessive vibration is encountered. The relationship of material resonant frequency ( $f_n$ ) with elastic modulus (E) and material density ( $p$ ) is as follows:

$$f_n \sim \sqrt{E/p}$$

By this relation, a Be/Ti composite with an  $E = 29 \times 10^6$  psi and  $p = 0.10$  lbs./cu.in. would have a 75% higher natural resonant frequency than steel, all other things being equal. The Be/Ti composite can thus safely operate at approximately 75% higher speeds and have the further advantage of weighing about one-third less than that of an equally sized shaft of steel.

Further possibilities in a fibrous Be/Ti composite fabricated by this invented process would be the "customized" array of Be fibers in the cross section. For instance: if a composite beam were to be desired which was subjected to bending in use, then a high population of continuous Be fibers could be placed in the outer area of the cross section so as to increase the elastic modulus selectively. Thus, the beam could very beneficially be stiffened by selective fiber placement in areas of maximum bending strain by selective concentrated use of Be fibers there. In less critical areas where bending strains were low less volume per cent of Be and more of Ti material could be employed to improve the ductility, toughness, impact strength and tensile strength in this area as well as lower overall cost. As a result of the opportunity to distribute location, size and proportion of continuous Be fibers and the proportion of continuous Ti material matrix, great flexibility in product property distribution exists and fibrous Be/Ti composite shapes can be customized in structure and properties so as to achieve maximum design goals, including stiffness, weight, strength, ductility, and toughness.

The present process eliminates many of the steps taught by the prior art, enables the utilization of commercial beryllium and commercial titanium materials without sacrificing raw material and processing savings. The present process further enables the use of higher hot working temperatures at which extrusion can be effected more readily allowing greater reductions, lower loads on tooling or fabrication of more complex shapes. Finally, the present process produces fibrous composite material of mechanical properties and ductility especially in the direction transverse to working higher than attained by a powder-powder composite process. The fibers of beryllium are continuous, that is, they extend in an axial direction, and preferably from end-to-end of the extruded member. As used herein the term "fiber precursor body" is intended to identify the form the beryllium component takes prior to extrusion after which it assumes a more nearly fibrous form than being of relatively small cross-sectional area, but very much elongated as well as fully densified due to the extrusion. The fiber precursors may be shaped as rods, bars, wires, etc. of varying degrees of density ranging from loose powder to fully densified beryllium.

The density and modulus of elasticity requirements above set forth are satisfied by beryllium/titanium composite containing from 40 to 60 volume percent beryllium, balance titanium or titanium alloy. The present invention, however, is also applicable to fibrous composites of beryllium and titanium outside of the 40 to 60% by volume beryllium for which uses may be contemplated in aircraft structures and elsewhere.

#### BRIEF STATEMENT OF THE INVENTION

Briefly stated, the present invention is in a process for producing and a product produced by forming an extrudable beryllium/titanium assembly of discrete beryllium fiber precursor bodies extending from end-to-end of said assembly; filling the balance of the assembly with titanium or titanium alloy to form a continuous matrix surrounding said bodies; encasing the assembly in an extrusion cannister and extruding the cannister at a temperature of from 1,350° to 1,525°F at a reduction ratio of from 6:1 to 100:1 or greater to form a solid fibrous beryllium/titanium composite.

In a more detailed embodiment in accordance with the present invention the following steps are included.

1. Designing the array configuration of Be fibers to be achieved in the final solid extruded Be/Ti composite shape.

2. Relating this configuration back to the necessary extrusion billet array configuration.

3. Assembly of an extrusion billet inside a steel cannister of one-sixteenth inch to one-half inch thick wall having the desired array configuration. This in terms of input material may consist of the following:

##### a. Be preforms — Ti powder

In this instance, Be preform fiber precursor bodies made from wrought Be or some form of rigidized or consolidated powders are maintained in a desired array by mechanical means or adhesive fixturing. The Be preforms are then surrounded by a material of Ti powder poured in around the preforms and the powder vibrated or tamped to as high a density as possible. Additional powder may be placed in the ends of the extrusion billet to supply additional volume of the low density powder which will flow in place during hot extrusion. (See FIG. 2.)

##### b. Solid Ti — Be powder or preforms

Alternatively the Ti material component may be a solid cast or wrought body processed commercially into which holes have been machined or otherwise prepared to receive the Be component. These holes can be filled with Be powder as the fiber precursor body which can be at least partially consolidated by vibration, tamping or cold pressing.

##### c. Be powder—Ti powder

Another alternative is that both the titanium and beryllium be in powder form. In this instance a thin separator such as plastic tubing or paper of the proper diameter is held in the desired way by mechanical means. Ti powder is poured around the thin wall plastic tubing and Be powder is placed inside the thin wall plastic tubing. The assembly is then vibrated or tamped to as high a density as possible. The thin-wall separator is then mechanically removed.

Aluminum or Ti or Ti alloy thin-walled tubing can also be used as separators. In this instance, the separators may remain in place and alloy with either the Ti or Be during subsequent processing.

4. The canned extrusion billet assembly having the desired array of Be and a Ti matrix may then be outgassed at 600° to 1,300°F. in the presence of a suitable vacuum of approximately 0.1 micron of Hg absolute pressure (optional).

5. The extrusion billet assembly may be cold pressed or isopressed at 5,000 – 60,000 psi before extrusion. Isostatic pressing may so distort the can as to necessitate the removal of the compacted body, machining to desired size and recanning (optional).

6. The canned or re-canned billet is heated uniformly up to the desired extrusion temperature of 1,350° to 1,525°F. and held for a minimal time period.

7. The heated billet is then extruded to at least a 6/1 reduction ratio and up to approximately 50/1 reduction ratio using commercial hot extrusion techniques.

8. The extruded solid Be/Ti composite is cooled to room temperature and stripped from its steel jacket by mechanical means or pickling in nitric acid.

9. When extrusion reduction ratios upwards of 20/1 are desired, it may be found convenient to re-extrude the jacketed billets at the same elevated temperature above 1,375°F using portions of clad extruded rod or shape. Alternatively, the cladding may be stripped, and the beryllium/titanium composite re-jacketed for further reduction in cross-sectional area. In this latter case, bundles of previously extruded and dejacketed composite rod or shapes may be both further reduced in cross section and metallurgically bonded together in this secondary extrusion operation.

10. Resultant extruded beryllium/titanium composite material after cooling to room temperature may be cold worked at 70% to 80% of ultimate tensile strength in order to remove normal residual tensile stresses present in the beryllium phase due to incompatibilities in contraction and modulus of elasticity and to impose a new residual compressive stress on the beryllium phase. With such prestressing, the material then elastically deforms in tension according to its true modulus of elasticity which is in the range of from 26 to  $32 \times 10^6$  pounds per square inch up to high stress levels. The 0.2% offset yield strength, an important engineering design parameter, has then been substantially raised.

45 It is here again pointed out that the processing temperatures of the present invention are generally higher than those previously used for the reason that hot working processes such as extrusion are facilitated. By this is meant that pressures required to extrude decrease with higher temperature, and greater reduction of cross section can be effected for equivalent pressures at 1,350° – 1,525°F as compared to 900° – 1,300°F used in prior art. For equal reduction ratios lower pressures are required, resulting in longer tool life. It has been found that beryllium/titanium composites hot extruded at 1,350° – 1,525°F exhibit a tensile strength comparable to or greater than those extruded at lower temperatures, but greater ductility than those extruded at 1,300°F and below. A titanium beryllide structure has been metallographically identified between contacting beryllium and titanium particles when the composite is extruded at 1,350°F and higher. Development of this phase may result in a stronger bond providing greater strength and ductility. Material extruded at 1,525°F and above exhibits lower strength and ductility perhaps because the interparticle titanium beryllide structure has grown excessively thick.

55 60 65 60 65

## BRIEF DESCRIPTION OF DRAWINGS

It becomes convenient to illustrate the process and resulting products produced in accordance with the present invention by specific examples, and in this connection reference may be had to the drawings which illustrate specific arrays of beryllium fiber precursor bodies in titanium matrices, and specific cannistered assemblies, and wherein:

FIG. 1 is a diagrammatic and schematic cross-sectional view of an array of beryllium rods of two different diameters arranged on and supported on a mild steel disc. The interstices will be filled with titanium alloy powder to form the extrusion assembly.

FIG. 2 is a diagrammatic and schematic cross-sectional view of a canister prior to extrusion.

FIG. 3 shows diagrammatically and schematically an array useful in making a hollow fibrous beryllium reinforced titanium composite shaft.

FIG. 4 shows diagrammatically and schematically a cross-sectional view of a cannister for a hollow shaft prior to extrusion.

FIG. 5 shows diagrammatically and schematically a cross-sectional view of an extrusion assembly of beryllium bars in a titanium matrix, the bars being arranged in a star pattern.

## DETAILED EXAMPLES OF INVENTION

The present process contemplates the use of commercially produced and readily available beryllium and titanium materials including powders, solid shapes and alloys. This is in contradistinction to specially produced powders such as the microquenched, age-formed, "shot" powders of the prior art.

The beryllium used in accordance with this work is commercially available and comes from a vacuum-cast metal source. Beryllium powder is comminuted by chipping vacuum-cast billets and grinding by known procedures. Solid beryllium preform shapes useful as fiber precursors are fabricated from powders, preferably containing from 0.2% to 6% by weight BeO, usually by the widely used commercial process of vacuum hot processing, and resultant dense bodies are then machined into desired Be preform shapes. Alternatively, preform shapes from beryllium powder can be fabricated by either cold pressing alone, or by cold pressing and sintering in vacuum at 1,150° - 1,250°C or by cold pressing, sintering and coining at room temperature up to 1,200°F. (and optionally resintering). Finally preform shapes from beryllium powder can be made by mixing with common binders to achieve porous but handleable fiber precursor bodies. Preform shapes can also be obtained from commercially available wrought forms of Be including extrusions, sheet metal or forgings. It is such preform shapes, e.g. rods, bars, wire, etc., which are preferably used as beryllium fiber precursors in fabricating the composites of the present invention.

The titanium material used in this process consists of both powders and solid material. Titanium materials may consist of up to 100% Ti or a commercially available powdered titanium alloy. These powders may be produced commercially by the conventional hydride-dehydride process which is well known, or by other commercial processes. Generally, these powders have a particle size in, or particle size distribution over, the range of from -20 mesh to +325 mesh, and preferably

no more than  $3 \times 10^{-2}$  inch. The solid Ti material also used in the present process can be up to 100% Ti or of commercial Ti alloy composition. Such solid Ti material is commercially available in a vacuum arc cast and wrought form in a wide variety of shapes and sizes adaptable to use in this process.

## Example No. 1

## (50 Be/50 Ti by volume Fibrous Composite)

## 1. Material Input

Be-Vacuum hot pressed Be powders of full density extruded and machined into  $\frac{1}{4}$  inch dia. (10 each) and  $\frac{3}{8}$  inch dia. (61 each) rods.

Ti-6Al-4V alloy powder of hydride derivation and of -50 +325 mesh size.

## 2. Array Configuration in Extrusion Billet. See FIG.

1. There is here shown a plurality of beryllium rods held in a drilled circular mild steel disc 0.5 inch thick and 4.480 inches in diameter, the larger diameter rods being arranged at the apices of equilateral triangles. The free space is ultimately filled with the titanium alloy powder.

## 3. Extrusion Billet Assembly

A. With reference to FIG. 2, there is shown diagrammatically an extrusion canister. The canister is composed of a plug 10 having integral therewith a drilled plate 12 into which the prefabricated beryllium rods 14 are inserted as indicated in FIG. 1. Welded to the plug 10 is a steel tubular body 16 having a wall thickness of approximately 0.25 inch and, in the specific example involved, being 5 inches in outside diameter. This is made of mild steel. As indicated, the titanium alloy powder fills the spaces between the beryllium rods 14 and, because of its powder condition, extends beyond the extremities of the beryllium rods. The canister is sealed with a plug 18 drilled to provide an exit bore 20 and having a stainless steel evacuation tube 22 welded thereto. The evacuation tube is to enable removal of gases from the interior of the canister after which it is sealed.

4. Extrusion Cannister outgassing — Evacuated to 0.1 micron of Hg.

5. Extrusion temperature — 1,425°F

6. Extrusion ratio — 15.7 (5 inches dia. to 1.25 inches dia.)

## 7. Extruded properties

| Property    | As Extruded |         | Prestressed to 96 ksi (tension) |
|-------------|-------------|---------|---------------------------------|
|             | Long.       | Transv. |                                 |
| $F_y$ , ksi | 53          | —       | 100                             |
| $F_u$ , ksi | 128         | 66      | 130                             |
| $e_t$ , %   | 4.3         | >1      | 4.0                             |

## Example No. 2

## (50% Be/50% Ti by volume) — Fibrous Composite

## 1. Material Input

Be-Vacuum hot pressed to powder of full density extruded and machined into  $\frac{1}{4}$  inch dia. rods.

Ti - Ti - 6Al - 4V alloy powder of hydride derivation and of -50 +325 mesh size.

2. Array configuration in extrusion billet similar to FIG. 1, but billet size 1 1/4 inches dia.  
 3. Extrusion billet assembly  
 Similar to FIG. 2, but billet 1 1/4 inches dia.  
 4. Extrusion cannister outgassing — none.  
 5. Extrusion temperature — 1,375°F.  
 6. Extrusion ratio — 20/1 (to 0.39 inch dia. composite).  
 7. Properties

| Property        | As Extruded |         | Prestressed to 72 ksi (tension) |
|-----------------|-------------|---------|---------------------------------|
|                 | Long.       | Transv. | ksi Long.                       |
| Tensile         |             |         |                                 |
| $F_{t_y}$ , ksi | 55          | —       | 75                              |
| $F_{t_u}$ , ksi | 96          | —       | 98                              |
| $e_t$ , %       | 1.0         | —       | 1.0                             |
| 3 Pt. Bend Test |             |         |                                 |
| $F_b$ , ksi     | <240        | —       | —                               |
| $e_b$ , %       | <10         | —       | —                               |

## Example No. 3

(50 Be/50 Ti by volume fibrous composite)

1. Comment — Example No. 3 is the re-extruded product of Example No. 1.  
 2. Extrusion billet — 1 1/4 inches dia. composite of Example 1 jacketed in a 1 1/4 inch OD  $\times$  1 1/4 inches ID steel tube.  
 3. Extrusion temperature — 1,450°F.  
 4. Extrusion Ratio — 20/1  
 (composite 1 1/4 inches dia. to 0.28 inch dia.).  
 5. Extruded properties.

| Property        | As Extruded |         | Prestressed to 100 ksi (tension) |
|-----------------|-------------|---------|----------------------------------|
|                 | Long.       | Transv. | Long.                            |
| Tensile         |             |         |                                  |
| $F_{t_y}$ , ksi | 53          | —       | 110                              |
| $F_{t_u}$ , ksi | 143         | 90      | 148                              |
| $e_t$ , %       | 4.5         | —       | 4.3                              |
| 3 Pt. Bend      |             |         |                                  |
| $F_b$ , ksi     | 276-356     | —       | —                                |
| $e_b$ , %       | 14          | —       | —                                |

## Example No. 4

(50% Be/50 to Ti by volume Fibrous Composite)

1. Material Input  
 Be-Vacuum hot pressed Be powder to full density extruded and machined into 0.445 inch dia.  $\times$  14 inches long rods (24 each). Ti - 6Al - 4V alloy powder of hydride deviation and of -50 +325 mesh size.  
 2. Array configuration in extrusion billet. See FIG. 3.

- B. In this example, the arrangement of the beryllium rods is shown in FIG. 3. Thus, beryllium rods 24 are mounted in a base 26 formed of mild steel in a circular pattern. In the specific example, the outside radius of the plug portion 26 is 2.25 inch, the inner radius is 1.625 inches, and the centers of the beryllium rods 24 are disposed on a radius of 1.937 inch.

lium rods 24 are disposed on a radius of 1.937 inch.

## 3. Extrusion billet assembly

C. With reference to FIG. 4, there is provided a nose plug 26 which carries the beryllium rods 24 as indicated in FIG. 3. The canister generally indicated at 28 is provided with a tubular body 30 and carries a center core 32. The interstices between the beryllium rods and the center core 32 are filled with titanium alloy powder 34 as above indicated. A tail plug 36 encloses the canister and includes a tubular member 38 extending therethrough for evacuating the system and ultimate sealing. The extrusion canister of FIG. 4 is approximately 22.5 inches long and the elements are formed except where indicated of hot rolled steel. The canister is 5 inches in diameter and the walls 0.25 inch thick.

4. Extrusion Cannister outgassing 0.1 $\mu$   
 5. Extrusion temperature 1425°F.  
 6. Extrusion ratio 20/1  
 7. Extruded properties

| Property        | As Extruded |         | Prestressed to 100 ksi (tension) |
|-----------------|-------------|---------|----------------------------------|
|                 | Long.       | Transv. | Long.                            |
| 3 Pt. Bend Test |             |         |                                  |
| Ult. strength   |             |         |                                  |
| $F_b$ , ksi     | 260         | —       | 271                              |
| Yield strength  |             |         |                                  |
| ksi             | 88          | —       | 188                              |
| Elong., %       | 4.6         | —       | 4.2                              |

## EXAMPLE NO. 5

A 4 1/2 inches OD, 3 1/2 inches ID Ti 6Al-4V tube was filled with -50 +100 mesh Be powder make 50% volume and canned, outgassed, extruded at 11 to 1 and 1,450°F. The product of this extrusion was re-extruded at 20:1 (~.306 rods). These rods were decanned, cleaned, bundled together, and re-extruded at 20:1 and 1,450°F. Resultant properties:

| As Extruded | As Extruded |           |
|-------------|-------------|-----------|
|             | $F_{t_y}$   | $F_{t_u}$ |
|             | 153 ksi     |           |
|             | 66 ksi      | 3 %       |

## EXAMPLE NO. 6

Be powder of -50 +100 mesh was cold pressed at 10,000 psi into 0.30  $\times$  0.22 inch cross-section rectangular bars. These bars were assembled into a can and surrounded by Ti-6Al-4V powder as shown in the FIG. 5:

- D. With reference to FIG. 5, there is shown diagrammatically and schematically another arrangement for beryllium bars 40 having the spaces therebetween filled with titanium powder 42. In general, the structure of the canister is essentially the same as shown in FIGS. 2 and 4.

The can was outgassed and extruded at 1,450°F. 20:1 resultant properties:

| As Extruded | As Extruded |           |
|-------------|-------------|-----------|
|             | $F_{t_y}$   | $F_{t_u}$ |
|             | 159 ksi     |           |
|             | 60 ksi      | 4.7 %     |

The impact resistance of Be/Ti fibrous composites is markedly superior to monolithic Be when both are measured by the well known Charpy test. The exact extent to which these composites resist impact (measured as standard Charpy V-notch) is dependent on the final size of the fibers in the composite. For instance, in Example 1 the fiber size was coarse and Charpy was 5.9 foot-pounds. The re-extruded product of Example 1 in which the fibers were of 1/10 of Example 1 was also tested. The Charpy impact in this case increased to 8.8 foot-pounds.

The method of achieving the fiber precursor has been found to have little bearing on impact performance. This is evidenced by impact performance similarities between Examples 1 and 5 for similar size fibers.

- alloy powders of hydride derivation. -20 mesh particle size or smaller and fractions thereof.
2. Primary densification data is listed below
  3. Array configuration — varied
  4. Extrusion billet assembly — varied
  5. Extrusion cannister outgassing — varied
  6. Extrusion ratio — 6:1 to 50:1
  7. Extrusion temperature — 1,350° - 1,525°F
  8. Properties
- 10 For given metal compositions under uniform conditions of extrusion, it has been found that the type of Be material and Ti material or its form used had little significance in respect to the longitudinal properties measured in the direction of extrusion of the extruded fibrous composite product. That is to say, whether dense
- 15

Combinations of Be and Ti Material Forms Used to Assembly Extrusion Billet for Composites

|                                                           | Ti & Ti Alloy Powder<br>Vibrated or Tamped | Ti & Ti Alloy Powder<br>Cold Pressed (Inc. Isostat.) | Solid Ti & Ti Alloy |
|-----------------------------------------------------------|--------------------------------------------|------------------------------------------------------|---------------------|
| Vibrated or tamped Be powder                              | X                                          | X                                                    | X                   |
| Pressureless sintered Be powder                           | X                                          | X                                                    | X                   |
| Cold pressed (including isostatic) Be powder              | X                                          | X                                                    | X                   |
| Cold pressed (including isostatic) and sintered Be powder | X                                          | X                                                    | X                   |
| Vacuum hot pressed (VHP) Be                               | X                                          | X                                                    | X                   |
| Wrought VHP Be                                            | X                                          | X                                                    | X                   |

Material and processing information relative to making extrusion billets having desired arrays of Be shapes in a Ti matrix are listed below:

1. Materials

- a. Be powder — commercial attritioned powder of -20 mesh particle size or smaller and screened or classified fractions thereof. In general, the particle size range is desirably controlled to be within a relatively narrow particle size distribution in a given sample, e.g. all under 50 mesh.
- b. Ti powder — commercial Ti and Ti - 6Al - 4V, Ti - 5Al - 2.5Sn, Ti - 6Al - 2Sn, and other titanium

extruded VHP Be rod, machined rod, or some form of porous compacted powder was used to form an array in the Ti matrix, the resultant extruded fibrous composite had similar longitudinal mechanical properties provided the final composite had an identical array and full densification of the beryllium as well as the titanium was accomplished.

Properties achieved rather than being dependent upon initial material form and density were related significantly to the temperature of extrusion, the extrusion ratio and the chemical (Beo content) and/or physical (particle size) composition of the Be and Ti materials.

| Forms of Be                                                          | Compaction Pressure | Approx. Sintering Temp. | Approx. Density % of Theo. |
|----------------------------------------------------------------------|---------------------|-------------------------|----------------------------|
| a. Vibrated powders                                                  | 0                   | —                       | 55                         |
| b. Pressureless sintered Be Powder                                   | 0                   | 1200°C                  | 95                         |
| c. Cold pressed powders or cold isopressed powders                   | 10-30 tsi           | —                       | 75                         |
| d. Cold pressed sintered powders or cold isopressed sintered powders | 10-30 tsi           | 1100°-1200°C            | >95                        |
| e. Vacuum hot pressed Be                                             | 500 - 1000 psi      | 1000°-1100°C            | >99.5                      |
| f. Wrought VHP Be                                                    | 500 - 1000 psi      | 1000°-1100°C            | 100.0                      |

Bearing this in mind, the following properties were achieved by extruded composites of 50 - 60% by volume Be fibers in a Ti material matrix:

| Low End of Range Properties           |                                                  |
|---------------------------------------|--------------------------------------------------|
| Conditions                            | Properties<br>(Longitudinal Direction)           |
| Low extr. temp. <1400°F               | $F_{t_y}$ (prestressed) 60-80 ksi                |
| Low extr. ratio <12:1                 | $F_{t_u}$ 90 - 115 ksi<br>$e_t$ 0.5-3.0%         |
| Be powder low in oxide,<br><2% Beo    |                                                  |
| High End of Range of Properties       |                                                  |
| High extr. temp. 1400-1525°F          | $F_{t_y}$ (prestressed) 80-100 psi               |
| High Extr. ratio >12:1                | $F_{t_u}$ 115 - 140 psi<br>$e_t$ >4%             |
| Be powder high in oxide<br>2 - 5% Beo | $F_b$ 250 - 300 ksi<br>$e_b$ 1 - 6%<br>$e_b$ >6% |

Properties in the direction transverse to extrusion were additionally dependent upon the ellipticity of the Be fibers. For instance in the case of extruded fibrous Be-Ti composites in which the Be fiber was cross-sectionally equi-axed, the  $F_{t_u}$  (transverse) was approximately 30,000 to 60,000 psi, where the ratio of width to thickness increased to 8 or greater, the transverse  $F_{t_u}$  increased to 100,000 psi.

What is claimed is:

1. A process for forming a solid fibrous composite from beryllium and titanium in which the titanium material forms a continuous matrix surrounding elongated beryllium fibers which comprises the steps of:

a. forming an extrudable beryllium/titanium assembly of:

1. discrete elongated beryllium fiber precursor bodies extending axially of said assembly;

2. filling the balance of the assembly with titanium to form a continuous titanium matrix surrounding said bodies;

b. encasing said assembly in an extrusion canister; and

c. extruding said canister at a temperature of from 1,400° to 1,525°F. at a reduction ratio of from 6:1 to 100:1 to form a solid fibrous beryllium/titanium composite.

2. A process in accordance with claim 1 which also includes the step of prestressing the extruded composite.

3. A process in accordance with claim 1 in which the beryllium fiber precursor is formed from beryllium powder having a particle size no greater than  $3 \times 10^{-2}$  inch.
5. A process in accordance with claim 1 in which the beryllium has a beryllium oxide content of from 0.2% to 6% by weight.
5. A process in accordance with claim 1 in which the beryllium fiber precursors are composed of vacuum hot pressed beryllium.
6. A process in accordance with claim 1 in which the beryllium fiber precursors are composed of cold pressed beryllium powder.
7. A process in accordance with claim 1 in which the beryllium fiber precursors are composed of cold pressed and sintered beryllium powder.
8. A process in accordance with claim 1 in which the beryllium fiber precursors are composed of cold pressed, sintered and coined beryllium powder.
- 20 9. A process in accordance with claim 1 in which the beryllium fiber precursors are composed of beryllium powder rigidized with a binder.
10. A process in accordance with claim 1 in which the titanium is in the form of a -20 +325 mesh powder.
- 25 11. A process in accordance with claim 10 in which the titanium powder has a particle size of no more than  $3 \times 10^{-2}$  inch.
- 30 12. A process in accordance with claim 1 in which the titanium is at least partially consolidated titanium powder.
13. A process in accordance with claim 1 in which the titanium is in the form of solid cast or wrought titanium metal.
- 35 14. A process in accordance with claim 1 in which the titanium material is titanium alloy.
15. A process in accordance with claim 14 in which the titanium alloy is Ti-6Al-4V alloy.
- 40 16. A process in accordance with claim 14 in which the titanium alloy is a Ti-5Al-2.5Sn alloy.
17. A process in accordance with claim 1 which also includes the step of degassing the extrusion canister to less than 10 microns of mercury.
18. A process in accordance with claim 1 which includes the step of isopressing the extrudable assembly at a pressure of 30 ksi prior to extrusion.
- 45 19. A process in accordance with claim 1 in which the extrusion canister is formed of low carbon steel.
- 50 20. A process in accordance with claim 1 in which the volume percent of beryllium is from 40% to 60%, and the balance is titanium or titanium alloy.

\* \* \* \* \*

UNITED STATES PATENT OFFICE  
CERTIFICATE OF CORRECTION

Patent No. 3,821,841

Dated July 2, 1974

Inventor(s) Vernon L. Goodwin

It is certified that error appears in the above-identified patent and that said Letters Patent are hereby corrected as shown below:

Column 7, line 56, "to" should be --of--.

Column 8, line 52, "retangu=" should be --rectangu- --.

Column 9, last line, "Ti - 6Al - 2Sn" should be

--Ti - 6Al - 6V - 2Sn,--.

Column 10, line 47, "(BeO content)" should be --(BeO content)---.

Column 11, in the table, line 16, "80-100 psi"

should be --80-100 ksi--; and

line 17, "115-140 psi" should be --115-140 ksi--.

Signed and sealed this 18th day of February 1975.

(SEAL)

Attest:

RUTH C. MASON  
Attesting Officer

C. MARSHALL DANN  
Commissioner of Patents  
and Trademarks